

Sept. 4, 1923.

1,467,037

J. H. HIRT

CHLORIDIZING OF ORES

Filed Jan. 10, 1920

Fig. 1,



Fig. 3,



Fig. 2,



Fig. 4,



Jules Weitac Hirt Inventor  
By his Attorneys  
Kunis, Guis, Marano & Edwards

Patented Sept. 4, 1923.

1,467,037

# UNITED STATES PATENT OFFICE.

JULES HECTOR HIRT, OF EL PASO, TEXAS, ASSIGNOR TO ALVARADO MINING AND MILLING COMPANY, OF NEW YORK, N. Y., A CORPORATION OF MAINE.

## CHLORIDIZING OF ORES.

Application filed January 10, 1920. Serial No. 350,576.

To all whom it may concern:

Be it known that I, JULES HECTOR HIRT, a citizen of the United States, residing at El Paso, in the county of El Paso, State 5 of Texas, have invented certain new and useful Improvements in the Chloridizing of Ores; and I do hereby declare the following to be a full, clear, and exact description of the invention, such as will enable others 10 skilled in the art to which it appertains to make and use the same.

This invention relates to an improved process of chloridizing ores, concentrates, and other metallurgical products, to convert the 15 metal values into chlorides or oxy-chlorides which can be subsequently recovered, for example, by leaching. It is a characteristic advantage of the invention that the chloridizing operation is effected without 20 objectionable losses of metal values by volatilization or decomposition of the chlorides or oxy-chlorides.

The chloridizing of gold, silver, or copper ores is recognized to be a difficult and 25 delicate operation because of the losses which tend to take place, by volatilization or decomposition, if the temperature is too high, the volatilized chlorides escaping and being lost or being decomposed into insoluble 30 metal values which resist the subsequent leaching operation. It has accordingly been proposed to carry out the chloridizing of the ores at a temperature below the melting point of sodium chloride, that is, at temperatures 35 below about 800° C., and even at temperatures far below this, inasmuch as certain of the metal chlorides have a much lower melting temperature; and it has been proposed to effect the chloridizing of the ore 40 by subjecting the mixed ore, usually a sulfide ore, and chloride, to oxidizing conditions, such as result from the introduction of air or of products of combustion, so that the sodium chloride or other chloride would 45 be decomposed to form chlorine as the effective chloridizing agent. Such processes are of limited applicability, because of the low temperatures required to prevent loss by volatilization, and the objectionable high 50 losses that take place if higher temperatures are employed.

According to the present invention, the objections incident to such prior proposals are largely overcome and the chloridizing operation is effected without objectionable

loss of metal values by volatilization or decomposition.

I have discovered that if a body or column of crushed ore is caused to pass through a closed or sealed atmosphere of heated 60 chloride vapors, not only can the volatilization losses be substantially eliminated, but the temperature can be varied between rather wide limits. I have further discovered that this process can be advantageously carried out with non-sulfide ores, so that sulfur 65 or sulfides are not present or required to generate the chloridizing atmosphere from the chlorides.

One type of furnace adapted for use in 70 the practice of the invention as shown in the accompanying drawing in which Figure 1 is a vertical section of the furnace; Figure 2 is a similar section in the plane transverse to the plane in Figure 1; Figure 3 is a vertical 75 section through the heating flues; and Figure 4 is a section at the line 4—4, Figure 3.

The improved process of the present invention can be carried out in different ways, and in different types of apparatus, provided the ore body is subjected to the chloridizing action of the vapors of sodium chloride (or its equivalent). The ore may thus be fed into a reaction chamber containing vaporized sodium chloride, and heated 80 in such chamber to the necessary temperature for the chloridizing reaction. I have found that a particularly advantageous manner of carrying out the improved process is to mix the ore, crushed to a suitable 85 size, with the proper percentage of sodium chloride or other chloride, such as calcium chloride, magnésium chloride, or iron chloride, and progressively feed the resulting mixture into an upright or vertical retort or chamber, and to heat the mixture therein to a sufficient temperature and for a sufficient time, to bring about the desired chloridizing of the metal values. The upright 90 or vertical retort or chamber 5 may advantageously be of rectangular cross-section and of a construction similar to that of coke-ovens, but made of materials resistant to the chemical action of the materials undergoing reaction therein, for example, of firebrick. 95 These upright or vertical retorts or chambers may thus be made of firebrick and with flues 6 in their side walls, with provision for example, burners 7 for heating the retorts or chambers at their central portions, or for 100

105 110

a sufficient portion of their length. It is desirable not to extend the heating flues for the entire height of the retorts, or, if the flues extend for the entire height, it is preferable to so regulate the heating action that the upper and lower ends of the retorts will not be heated. The cold air may thus be drawn in through inlet 8 to the flues near the bottom of the retort or chamber and thereby preheated by the material that has undergone treatment and is passing out through the lower part of the retort. Similarly, the hot products of combustion may be advantageously passed to a stack 9 through the flues at the upper part of the retort or chamber to preheat the incoming mixture.

When the retort or chamber has been once charged, the process becomes continuous, and requires merely the charging of further amounts of the mixture of ore and chloride at the top and the discharging of the cooled chloridized ore at the bottom through a chute 10 which is provided with a closure 11. The ore itself forms an effective seal for the retort or chamber, inasmuch as the cooler portions of the ore at the inlet end of the chamber effectively condenses any chloride vapors and carries them back into the reaction zone. The cooled chloridized ore at the lower end of the retort or chamber similarly prevents escape of chloride vapors, although there is relatively little tendency for these vapors to escape with the ore at the bottom, inasmuch as the vaporized chlorides tend rather to rise to the upper parts of the retorts or chambers. As the mixture of ore and salt reaches the heated reacting zone, the sodium chloride melts and becomes vaporized so that the reaction zone of the retort or chamber contains a more or less saturated atmosphere of the vaporized chloride. This insures that all parts of the ore are subjected to the action of the vapor, and thorough chloridizing of the metal values as they pass through the hot chloride vapors and are brought into reactive contact therewith.

In a furnace construction of the character above described, that is, a vertical or upright retort or chamber, or a series of such retorts or chambers, heated by conduction through flues in the side walls thereof, the charge passing through the furnace is subjected to preheating as it enters the upper parts of the retorts or chambers, and the preheated charge is then subjected to the reaction zone, the reaction being promoted by the preheating of the charge. After the reaction, the chloridized ore then passes down through the cooling zone where it serves to preheat the air for combustion. The heating of such furnaces can be effected with oil or gas as the fuel in a manner which will be readily understood. In such a furnace, as above pointed out, the cold de-

scending ore entering the retorts or chambers forms an effective seal preventing any tendency of the hot chloride vapors to escape through the top of the retorts or chambers. The chlorides are thus kept within the retorts or chambers until they have exerted their desired chloridizing action, and the products of this chloridizing action then escape from the bottom of the furnace. If a considerable excess of sodium chloride is used, this excess may pass away with the chloridized ore, but, inasmuch as the tendency is for the hot chloride vapors to rise and not to descend with the hottest ore as it travels through the zone of highest temperature, objectionable escape of the chloride in vapor form is effectively prevented, provided the chloridized ore is permitted to cool sufficiently before it is discharged from the furnace.

The process of the present invention, as above pointed out, is of particular value for the treatment of non-sulfide or oxidized ore, as distinguished from sulfide ores; although it is also applicable to the treatment of sulfide ores. Even low grade ores, that is, ores containing but a small percentage of metal values, can be effectively chloridized, and the values converted into chlorides or oxychlorides well adapted for the subsequent recovery thereof by leaching. Ores containing as high as 10% of copper have been effectively chloridized in this way. Ores relatively rich in gold and silver have likewise been effectively chloridized, and the gold and silver subsequently recovered from the chloridized ores.

The amount of the common salt (sodium chloride) or other chloride, such as calcium or magnesium chlorides or iron chloride, will vary somewhat with variations in the values contained in the ores to be treated. With gold and silver ores, it is of advantage to use only a relatively small amount of common salt or other chloride, for example, one per cent or less, and ores treated with such amounts of chloride are particularly well adapted for subsequent leaching by the cyanide process. In general, only a few per cent at most of the chloride will be required. Any excess is unobjectionable if the values are to be subsequently leached with a chloride solvent, inasmuch as the excess chloride used will assist in the subsequent leaching operation and will be thereby recovered. The chloride can be mixed with the ore in any suitable manner. The intimacy of intermixture can be promoted by using a solution of the chloride, but this will not usually be necessary because the chloride, even if added in a solid form, will be subsequently vaporized and will mainly react in its vapor state, so that thorough chloridizing will be effected.

Among the characteristic advantages of

the process may be mentioned the following. The ore does not require fine grinding, inasmuch as the intense penetrating effect of the hot chloride vapors insure penetration of even relatively coarse particles of the ore, if the ore is sufficiently porous. With many ores, it will not be necessary to grind finer than about  $\frac{1}{2}$  inch, whereas with processes heretofore proposed, in so far as I am aware, it has been customary to grind the ore to a fine state of subdivision. The sodium chloride or other chloride similarly does not require fine grinding or thorough mixing, but the required intimacy of intermixing and reaction is insured by the fact that the chloride is vaporized and is present in the reacting zone, in part at least, in vapor form. Furthermore, a minimum amount of the sodium chloride or other chloride is required, although any excess, not consumed, will pass through unchanged and may be recovered in the subsequent leaching operation. Even extremely high temperatures may not be objectionable, inasmuch as escape of the volatile chlorides is prevented, but such temperatures may even be advantageous in facilitating the reaction and shortening the time required. The temperature regulation thus becomes of less importance, although the temperature should, of course, be sufficient to insure rapid and effective chloridizing. No sulfur or sulfides are required in the ore to generate the chloridizing atmosphere; and, if sulfides are present, the ore is not subjected to atmospheric oxidation, but the reaction is brought about by the vaporization of the sodium chloride or other chloride which reacts in its vaporized condition with the metal values, although reaction may likewise take place to a greater or less extent directly with the molten sodium chloride, to the extent that it is present unvaporized in the reaction zone. Inasmuch as there is no flow of gases into and out of the reaction zone, there is no loss of volatile chlorides due to convection therewith.

The ore employed need not be previously dried, but may be used in a moist state, inasmuch as any moisture which it contains will be readily removed in the upper preheating zone of the furnace.

Instead of carrying out the process in furnaces of the construction above referred to, other suitable types of furnaces can be used which will enable the desired heating and reaction to be brought about. Horizontal or inclined heated chambers or retorts can thus be used, provided they are provided with suitable heating means for heating them to the proper temperature and with means for supplying thereto the ore and chloride and for removing therefrom the chloridized ore.

The temperature required for the process can, as above pointed out, be varied rather

widely, inasmuch as considerably increased temperatures will not cause objectionable loss of the volatile chlorides, or objectionable decomposition thereof. When common salt (sodium chloride) is used, which has a melting point of about  $804^{\circ}$ , the temperature should preferably be maintained around  $800$  to  $900^{\circ}$  or somewhat higher. With calcium or magnesium chlorides, which have a somewhat lower melting point, somewhat lower temperatures can be used.

The cold chloridized ore can be subsequently treated in any suitable manner for the recovery of the values therefrom. These values, in the form of chlorides or oxychlorides, are well adapted for recovery by leaching operations, for example, by leaching with cyanide solutions, with hyposulfite, with a saturated brine (sodium chloride) solution, with an acid brine solution (containing 1 or 2% of hydrochloric or sulfuric acid), a brine solution containing ferric chloride, etc. The methods of leaching the ore and of recovering the values from the resulting liquor will be readily understood and need not be further described.

I claim:—

1. The method of chloridizing ores, metallurgical products and the like, which comprises subjecting a body of ore fed at a rate which ensures the presence of a layer of cooler ore overlying the reaction zone, to the chloridizing action of an atmosphere containing the vapors of a suitable volatile chloride while protecting the same from atmospheric oxidation and preventing escape of volatile metal chlorides by condensing the latter in the overlying layer of cooler ore.

2. The method of chloridizing ores, metallurgical products and the like, which comprises mixing the ore with a suitable chloride, feeding the mixture at a rate which ensures the presence of a cooler layer overlying the reaction zone, heating the mixture while protected from atmospheric oxidation to a sufficient temperature to cause reaction between the chloride and the metal values of the ore, and preventing escape of the volatile metal chlorides by condensing the latter in the overlying cooler layer.

3. The method of chloridizing ores, metallurgical products and the like, which comprises mixing the ore with a suitable chloride, confining the mixture as a compact column in a suitable receptacle and heating the column intermediate its ends while protected from contact with the products of combustion to a sufficient temperature to effect the desired chloridization.

4. The method of chloridizing ores, metallurgical products and the like, which comprises progressively feeding a charge of ore admixed with a suitable chloride through a reaction zone at a rate which ensures the presence of a cooler layer overlying the re-

action zone, heating the mixture to a sufficiently high temperature to effect the desired chloridization and preventing escape of the volatile chlorides from the charge by condensing the latter in the overlying cooler layer.

5. The method of chloridizing ores, metallurgical products and the like, which comprises progressively feeding a charge of ore 10 admixed with a suitable chloride into a pre-heating zone and then into a reacting zone, heating the same in the reacting zone to the reacting temperature while protected from atmospheric oxidation, and subsequently 15 passing the chloridized ore through a suitable cooling zone, the preheating and cooling zones being arranged to prevent escape of volatile chlorides through the material contained therein.

20 6. The method of chloridizing ores, metal-

lurgical products and the like, which comprises establishing a body of such material admixed with a chloridizing agent and subjecting the body to heat from an external source at a zone intermediate its ends while 25 the ends are maintained in a cooler state.

7. The method of chloridizing ores, metallurgical products and the like, which comprises establishing a body of such material admixed with a chloridizing agent, subjecting the body to heat from an external source at a zone intermediate its ends, while the ends are maintained in a cooler state and advancing the body through said zone by the withdrawal of chloridized material at one 30 end and the addition of fresh material at the other.

In testimony whereof I affix my signature.

JULES HECTOR HIRT.